

# United States Patent Office

**3,392,046**

Patented July 9, 1968

1

3.392.046

**FIBROUS ORGANIC MATERIAL HAVING AFFIXED  
THERETO A POLYPERFLUORO ALKYL METH-  
ACRYLIC ESTER AND METHOD FOR MAK-  
ING SAME**

Herman Lowell Marder, Plainfield, N.J., assignor to  
Colgate-Palmolive Company, New York, N.Y., a cor-  
poration of Delaware  
No Drawing. Filed June 17, 1963, Ser. No. 288,442  
12 Claims. (Cl. 117—143)

## ABSTRACT OF THE DISCLOSURE

Fibrous organic material are rendered water, oil, stain and soil repellent by treatment with emulsions or solutions of perfluoro alkyl methacrylate polymers containing a terminal  $\text{CF}_3$  group.

The present invention relates to the preparation of omega-fluoro- or terminal  $-\text{CF}_3$  polymers of methacrylic acid and to the treatment of fibrous materials such as paper, leather, textiles and the like with the aforesaid omega-fluoro- or terminal  $-\text{CF}_3$  polymers.

The development of the principles of water repellency for obtaining textile materials which resist wetting by water cover the period of 1935 to 1940. Prior to that period, textile materials were coated with various compositions such as rubber, linseed oil-rubber mixtures, synthetic dopes, and other bizarre compositions which formed a continuous coating on the woven material and prevented water penetration.

Without understanding the basic principles of surface free energy, contact angle and spreading coefficient, several unrelated practical developments evolved during the period from 1935 to 1940 which changed the art of textile waterproofing. In Germany, especially at Chemische Fabrike Pferze, a series of paraffin wax emulsions was developed which, when padded onto textiles, produced a high contact angle of water drops on the surface and a high degree of shower resistance without changing the porosity or air permeability of the textile material. These treated fabrics were non-wettable by water or water borne liquids and stains because of the change in free energy of the fiber surfaces and not because of closing or plugging the holes in the interstices of the fabric.

By the use of the new wax emulsion-metallic salt compositions, it was then possible to produce fabrics which had the feel and appearance of conventional textiles, but did not look like oil-cloths, or rubberized coated fabrics. The only practical limitation of such compositions was the durability to washing and dry cleaning. Such products comprise generally a composition containing:

- (a) A paraffin wax or mixtures of vegetable wax esters such as carnauba, candillilla, or sugar cane wax.
  - (b) An emulsifying agent, generally glue, gelatin, and rosin soaps.
  - (c) An aluminum or zirconium salt, usually formates or acetates. The primary function of such salts is to insolubilize the glue and other emulsifiers after the emulsion is deposited on fabrics.

A large variety of such products are still in use as low cost non-durable water repellants for textiles. Since neither thermosetting nor reaction with the fiber occurs with such products, they all are non-durable to washing and dry-cleaning. Other than water repellency for rain wear fabrics, such products produce fabrics which have a fair degree of spot and stain resistance to water-borne stains.

The search for durable or relatively permanent water

2

repellents, especially for cellulosic fibers, evolved from the deficiencies of the wax emulsions. One of the first, if not the first, product to overcome the deficiencies of the wax emulsions was made available in Great Britain under the name of "Velan." This was octadecyloxymethyl pyridinium chloride, a quaternary ammonium compound made by the chloromethylation of octodecanol followed by quaternization with pyridine. This compound is unstable and under acid conditions reacts with surfaces containing active hydrogen, e.g., the hydroxyl group of cellulose fibers (ZOH) as indicated by the following formula:



Fabrics treated with such a compound are durably water repellent, are porous, soft, and appear like untreated fabrics. The stearamidomethyl analogue of "Velan" having a composition corresponding to the formula:



30 is known commercially as "Zelan" and "Norane R." The advantage of the stearamide product is greater initial water repellency and greater durability to washing. Such products are still leaders in rain wear fabric finishes.

Other fiber reactive and durable water repellents have been developed and are represented by silicone water repellents, methylol stearamide compositions, hydrophobic resins, octadecyl ketene dimer and others.

While durable water repellents had been developed initially for outerwear- and raincoat-type applications, in the period 1950 and 1956 such products began to be used widely on men's suitings, dress goods, and upholstery materials. It has been observed that fabrics treated with such durable water repellents have a high degree of soil resistance to water-borne soils and stains. However, a major limitation of such finishes is that they attract oily soils, and the fabrics are not stain repellent to oily materials such as oils, greases, gravy, mayonnaise, etc.

The fabrics treated with polymerized perfluoroalkyl esters of acrylic acid, e.g., those described in U.S. Patent No. 2,642,416, possess some of the advantages of the hereinbefore discussed durable water repellents plus the capability of resistance to staining by oil-borne stains. However, these polyacrylic acid esters are deficient in practical use since they are prone to enhance the tenacious adherence of particulate soil on the surface of the fabric. As a result, it is not practical to use these materials on white fabrics. For example, a garment treated with such materials, and rendered thereby oil and water repellent and resistant to liquid stains to a degree, would nevertheless be soiled in use by contact with particulate soiling materials so as to appear dirty and esthetically unacceptable. Therefore, it is evident that there are mechanisms of soiling involved, other than contact with staining liquids, in the practical use of repellent materials and the presently known materials are inherently self-defeating in this respect.

In contrast to the aforescribed deficiency of the poly-perfluoroalkyl esters of acrylic acid, it has now been found that all of the advantages of these repellents are retained and, in addition, the deficiencies of the aforesaid poly-acrylic acid esters are overcome by the use of the novel polymeric materials herein described. Fi-

brous materials are made repellent to particulate soils and the residue of the aforesaid particulate soil remaining on the fibrous material after conventional laundering is markedly reduced, by affixing to the fibrous material polymerized perfluoroalkyl esters of methacrylic acid.

The polyperfluoroalkyl esters of methacrylic acid have

Table II is a comparison of 2 HM-8 and 3 HM-7 polymeric coatings on 80 x 80 cotton fabric obtained by padding the fabric with 1% solutions of each polymer in 1,3-bis(trifluoromethyl)benzene, followed by drying to remove the solvent. The coatings exhibit the following characteristics:

TABLE II

| Polymer                   | Liquid Repellency Rating |        | Staining Characteristics |                |            |                |
|---------------------------|--------------------------|--------|--------------------------|----------------|------------|----------------|
|                           | Water Spray              | Oil    | Water Borne              |                | Oil Borne  |                |
|                           |                          |        | Repellency               | Launderability | Repellency | Launderability |
| (a) 2 HM-8.....           | 100                      | 100/90 | 6.4                      | 8.8            | 8.0        | 9.0            |
| (b) 3 HM-7.....           | 50/0                     | 0+     | 5.4                      | 8.4            | 4.8        | 6.8            |
| (c) Untreated Cotton..... | 0                        | 0      | 1.8                      | 5.4            | 1.8        | 5.6            |

compositions corresponding to the following repeating unit:



where F is fluorine and x is 1 to 20, preferably 2 to 12.

The monomer should be polymerized sufficiently so that it is not soft and tacky and should be substantially free from unconverted monomer and other low molecular weight telomers. The inherent viscosity which is a measure of the degree of polymerization will vary depending upon the particular fluorinated ester but will be usually within the range of about 0.2 to 3, and preferably at least about 0.5, said inherent viscosity being determined by the method described in Sorenson and Campbell, "Preparative Methods of Polymer Chemistry," Interscience Publishers, N.Y., 1961. The invention in its broadest aspect is not limited to this range since lower and higher polymers are useful also. In general it is considered that the number of repeating units (n) will be at least about 10 which can be illustrated by enclosing the above formula in brackets followed by the subscript "n".

The capabilities of these novel perfluoroalkyl esters of methacrylic acid having a terminal  $-\text{CF}_3$  group are to be distinguished from the capabilities of either (1) methacrylic acid esters having a terminal  $-\text{CHF}_2$  group or (2) acrylic acid esters having a terminal  $-\text{CF}_3$  group. The novel methacrylic acid esters having a terminal  $-\text{CF}_3$  group of the present invention endow the treated substrate or fabric with a more universal resistance to soiling than is given to fabrics or substrates by either acrylic acid esters having a terminal  $-\text{CF}_3$  group or the methacrylic acid esters having a terminal  $-\text{CHF}_2$  group. This is established by the data presented in the following tables using the test procedures described hereinafter involving comparisons of the properties of the polymers of the following three materials:



It will be noted that the 2 HM-8 polymer ( $-\text{CF}_3$  methacrylate) of the present invention is compared with 2 HA-8 (the corresponding acrylate) and 3 HM-7 (the  $-\text{CF}_2\text{H}$  methacrylate).

Table I is a comparison of the antisoiling properties of fabrics sized with emulsions of the polymethacrylate esters of fluorinated alcohols, i.e., 3 HM-7 and 2 HM-8 to yield approximately 2% by weight on the fabric:

TABLE I

| Polymer                   | Liquid Repellency Rating |     |
|---------------------------|--------------------------|-----|
|                           | Water Spray              | Oil |
| (a) 3 HM-7.....           | 70                       | 0+  |
| (b) 2 HM-8.....           | 70/0                     | 50  |
| (c) Untreated Cotton..... | 0                        | 0   |

It is apparent from the above data in Tables I and II that the 2 HM-8 polymer of the present invention confers markedly superior liquid repellency to water and especially oil as compared to the 3 HM-7 polymer under the same conditions as illustrated by the higher ratings in the liquid repellency tests.

Similarly, it is apparent from Table II that the 2 HM-8 polymer exhibits particularly unusual and effective anti-staining characteristics in comparison to the effects produced by the 3 HM-7 polymer (the higher the rating number approaching 10 means the greater the resistance to staining, and the higher the launderability number meaning the better removal of the stain).

Another unique property of the polymers of the present invention such as the 2 HM-8 is their resistance to particulate soil. As indicated, fabric treated with the corresponding poly-acrylate esters exhibit effective liquid repellency properties also, but these materials are particularly deficient in resistance to dry soil. The marked superiority of the methacrylate polymers of the present invention in comparison to the acrylate types is illustrated in Table III wherein the 2 HM-8 polymer is compared to the previously-described 2 HA-8 and to a commercial product having a polymer of a modified fluoroacrylate ester known as FC-208. For these tests, the cotton fabric is padded as described with a 2% concentration of the polymers and dried. The treated materials are subjected to staining by particulate oily dirt and the reflectance of the fabric is measured before and after washing, in comparison to an untreated control. In the table, a higher value indicates greater whiteness and therefore less staining of the fabric by the particulate soil.

TABLE III

| Polymer                     | "Dry Soil" Reflectance |                  |
|-----------------------------|------------------------|------------------|
|                             | Before Laundering      | After Laundering |
| (a) 2 HM-8.....             | 40                     | 74               |
| (b) 2 HM-8 (extra dry)..... | 43                     | 75               |
| (c) 2 HA-8.....             | 32                     | 58               |
| (d) FC-208.....             | 35                     | 44               |
| (e) Untreated Cotton.....   | 33                     | 78               |

The unusual properties of the fabric treated with the 2 HM-8 polymer of the present invention is self-evident from the data. The 2 HM-8 polymer-treated fabric, before laundering, exhibited much greater resistance to dry soil as compared to the untreated cotton as a control. In contrast, the fabrics treated with the 2 HA-8 and FC-208 materials exhibited no significant improvement in resistance to the particulate soil since their reflectance value before laundering were approximately the same as the untreated fabric.

The comparative reflectance values after laundering are particularly significant also. After washing, the fabric treated with the 2 HM-8 polymer was found to be as clean as the untreated cotton. In contrast, the fabrics treated with the acrylate polymers were found to be far dirtier than the untreated cotton indicating incomplete removal of the adsorbed soil to a substantial degree. Thus, these polymeric materials appear to promote retention of

particulate soil in addition to offering no resistance to its pickup on the fabric. A moment's reflection recognizes that the major mechanism of soiling is the dynamic contact of a clean surface, such as the neckband or the cuff of the sleeve of a man's shirt with a surface having thereon particulate soil such as the dust and dirt held on the neckband or cuff by the oily exudations of the human skin. Thus, a man's shirt treated with the other polymers indicated above will appear "tattle-tale grey" after washing, whereas a shirt treated with the 2 HM-8 polymer of the present invention will appear clean, white, and not "tattle-tale grey."

The data presented above clearly establish that although the difference in chemical structure between the novel perfluoroalkyl esters of the present invention in one comparison appears to be only the difference between an ester of acrylic acid and an ester of methacrylic acid and in the other instance the difference is between a terminal  $-\text{CHF}_2$  group and a terminal  $-\text{CF}_3$  group, nevertheless these differences appear to make the critical factor essential to superior universal or overall resistance to soiling, and particularly the difference between washed fabrics which are grey and washed fabrics having the white, clean appearance of untreated fabric.

The novel monomeric esters of the present invention are prepared by the classical methods of organic chemistry such as the esterification of methacrylic acid with the alpha, alphadihydroperfluoroalkanol [ $\text{CF}_3(\text{CH}_2)_x\text{CH}_2\text{OH}$ ] with distillation of the water produced or by reaction of methacrylyl chloride with the perfluoroalkanol in the presence of an acid acceptor or by the reaction of methacrylic anhydride with the perfluoroalkanol.

Thus, for example, 1,1-dihydropentadecafluoroctylmethacrylate was prepared from the following charge in the manner described hereinafter.

#### CHARGE

|                                                  |                   |      |
|--------------------------------------------------|-------------------|------|
| Methacrylic acid                                 | grams             | 17.2 |
| 1,1-dihydropentadecafluoroctyl alcohol (0.1 mol) | grams             | 40.0 |
| Hydroquinone                                     | do                | 0.1  |
| Concentrated sulfuric acid                       | cubic centimeters | 0.5  |
| Benzene                                          | do                | 85.0 |

#### EQUIPMENT

300 cubic centimeters flask equipped with a stirrer, a 45 Dean-Stark azeotrope apparatus, a condenser on the top of the Dean-Stark apparatus, with a thermometer.

#### PROCEDURE

(1) Charged reactants; heated eight minutes before 50 condensed water and benzene refluxed and accumulated in the trap. (In the following "log" consider the foregoing enumerated eight minutes as zero time).

| Time (minutes): | Cubic centimeters<br>water distilled |
|-----------------|--------------------------------------|
| 0               | 0.3                                  |
| 23              | 0.6                                  |
| 66              | 1.0                                  |
| 162             | 1.2                                  |
| 313             | 1.6                                  |
| 757             | 1.2.2                                |

<sup>1</sup> Theoretically only 1.8 cubic centimeters should have been produced in the complete esterification of the perfluoroalkanol. The excess water arises from the water in the reactants.

(2) Attached simple distilling head, thermometer and condenser, nitrogen capillary (no stirring) and water suction to the reaction flask. The reaction mixture was distilled at reduced pressure to obtain the following fractions:

| Fraction No. | Pressure,<br>mm. of Hg | Temper-<br>ature,<br>°C. | Weight,<br>gm. |
|--------------|------------------------|--------------------------|----------------|
| I            | 83-20                  | 43-85                    | 40.7           |
| II           | 20                     | 72-102                   | 8.3            |

(Water accidentally was introduced.) Fractions I and II were combined washed with water and redistilled with 0.05 grams of hydroquinone.

#### Weight of Fractions I and II—34.6 grams

| Fraction No. | Pressure,<br>mm. of Hg | Temper-<br>ature,<br>°C. | Weight,<br>gm. |
|--------------|------------------------|--------------------------|----------------|
| 2-1          | 20                     | 78-95                    | 21.1           |
| 2-2          | 20-21                  | 95-102                   | 10.3           |

Fraction 2-2 was practically 100 percent of the monomer, dihydropentadecafluoroctyl ester of methacrylic acid. Fraction 2-1 was a mixture of the alcohol and the aforesaid monomer.

Similar methacrylate monomers are prepared in like manner from other fluorinated alcohols having a similar structure such as the corresponding 1,1 dihydro butyl, nonyl, decyl and dodecyl alcohols and the like (all other hydrogens being replaced by fluorine).

The monomeric methacrylic acid esters of perfluoroalkanols having a terminal  $-\text{CF}_3$  group are polymerizable by known emulsion polymerization techniques employing anionic, non-ionic, and cationic surfactants. The method of polymerization may be by emulsion, solution or bulk, with ionic or radical catalysts. A preferred emulsion technique is exemplified by the following example:

#### CHARGE

|                                            | Grams |
|--------------------------------------------|-------|
| Deionized water                            | 28.00 |
| Sodium lauryl sulfate                      | 0.50  |
| Sodium tetraborate                         | 0.07  |
| 1,1-dihydropentadecafluoroctylmethacrylate | 14.00 |
| Potassium persulfate                       | .08   |

#### PROCEDURE

- Charged flask with all materials except the persulfate catalyst. Swept nitrogen through without agitation for 15 minutes. Heated contents of flask with stirring to 48.5° C. in 16 minutes.
- Added 0.04 gram of persulfate. In 40 minutes a trace of turbidity indicated initiation of the polymerization. Heated the contents of the flask for 68 minutes more and added 0.02 gram of persulfate.
- Heated contents of the flask 16 minutes more and added 0.02 gram persulfate. Heated contents of flask for three and a half hours more, and then cooled the flask and contents. Maximum temperature 50-55° C., total time—11.6 hours.
- Poured 35.4 grams of reaction emulsion into jar. The emulsion was calculated to contain 26.7 percent solids when dried to a hard polymer.

The polymer emulsion is usually dried at elevated temperature to remove the unconverted monomer. The 2 HM-8 polymer obtained is a hard, tough material which is non-rubbery and non-tacky at room temperature. This solid melts to form a clear viscous liquid when heated to about 550° F. Upon analysis, it corresponds to the structure:



and has an inherent viscosity of about 0.88 as measured in bis (tri-fluoromethyl) benzene for example.

Similar polymers are prepared from the previously described methacrylate monomers derived from the corresponding 1,1 dihydro butyl, nonyl, decyl and dodecyl fluorinated alcohols, and such polymers confer improved repellent properties when applied to the fabric as described.

#### Application to the substrate

The polymeric materials may be applied in any suitable manner. For example, the substrate, e.g. cotton, was

contacted with the finishes in a laboratory textile paddler in a conventional one dip- one nip to a wet pick-up of the desired concentration of finish. Thus, for a deposition of one percent of solids from a one percent concentration of solids in solvent or aqueous emulsion at a 90 percent wet pick-up the concentration of polymer in the aqueous emulsion or in the solvent is increased from one percent for 100 percent wet pick-up to 1/0.9 or 1.1 percent. Thus, for example, a known weight of 80 x 80 cotton print cloth (Style #400—test fabrics) was immersed in a known quantity of water and an aqueous emulsion of the polymer slowly added to provide the test concentration of polymer in the bath for an 80 to 90 percent wet pick-up. The bath was agitated for 10 minutes, the test cotton removed from the bath, and passed through the rollers once (one nip). The test cotton was then dried and cured at a temperature in the range of room temperature to about 375° F.

Alternatively, these polymerized perfluoroalkyl esters of methacrylic acid having a terminal  $-\text{CF}_3$  group also can be applied to the substrate from a solution in a solvent for the esters such as trifluoromethyl benzene, i.e., trifluorotoluene, hexafluoroxylene, aliphatic fluorooesters such as methylperfluoroacetate and similar perfluoro organic solvents. Presently, it is preferred to use trifluorotoluene as the solvent. For example, pentadecafluoroctyl methacrylate as a 1 percent solution in bis (trifluoromethyl) benzene was applied to cotton cured 10 minutes at 300° F. and subjected to the tests described herein after was found to exhibit excellent water-repellency, oil-repellency and dry stain repellency.

In general, the polymer is deposited from a liquid medium such as the aqueous emulsion so that the treated fibrous material has an elemental fluorine analysis in the range of 0.05 to 5%. The polymer is usually deposited on the fabric in an amount of 0.1 to 10% by weight of the fabric. The fabric treated with the polymeric materials may be dried in any suitable manner, including air-drying, i.e., room temperature of about 70-75° F., to about 375° F. It is preferred to air-dry followed by curing, though the curing may be of the wet fabric directly, at an elevated temperature in known manner such as up to about 375° F. for about 5 to 60 minutes, preferably about 200° to 375° F.

For rating the efficacy of a finish to provide (1) water-repellency, (2) oil-repellency, (3) dry-stain repellency, and (4) resistance to staining by water-borne stains and oil-borne stains, four procedures or tests are used.

#### Water repellency

This test is a modification of the "spray test" designated AATCC Standard Test Method 22-1952 to emphasize ratings when hydrophobic properties of the finish confine the area of wetting but permit wetting through. Thus, a spray rating number 70/0 indicates a 70 spray rating pattern. The "0" in the denominator indicates wetting to the under surface of the cloth at the wet areas but does not differentiate between small or large areas of wetting through.

The AATCC Standard Test Method 22-1952 is applicable to any textile fabric. It measures the resistance of fabrics to wetting by a water spray and the results depend primarily on the degree of hydrophobicity inherent in the fibers and yarns and the subsequent treatments applied. Water is sprayed against the taut surface of a test specimen. Evaluation of the wetted pattern is readily brought about by comparing the wetted pattern with standard wetting pattern pictures:

100—No sticking or wetting of upper surface

90—Slight random sticking or wetting of upper surface

80—Wetting of upper surface at spray points

70—Partial wetting of whole of upper surfaces

50—Complete wetting of whole of upper surfaces

0—Complete wetting of whole of upper and lower surfaces.

The test specimens of a minimum size of 7" x 7" are conditioned at 70° F. and 65 percent relative humidity for a minimum of four hours before testing.

The test specimen, fastened securely and wrinkle-free in a metal hoop having a diameter of 6 inches is placed and centered 6 inches under a standard spray nozzle at an angle of 45 degrees to the horizontal. Two hundred and fifty milliliters of water at 80±2° F. is poured into the funnel attached above the spray nozzle. The spray lasts 25 to 30 seconds at the end of which time the hoop is taken by one edge and the opposite edge tapped smartly once against a solid object with the wet side facing the solid; this procedure is repeated with the hoop reversed 180 degrees.

15

#### Oil repellency

This test is a modification of the test described in the publication of the Minnesota Mining and Manufacturing Company "3M Textile Chemicals" Appendix A, Test Methods, page 1.

20

The modification is concerned with a refinement of the rating system. The oil repellency rating in the numerator refers to the normal 3M rating system. The number in the denominator refers to the highest rated drop not wet through as observed when turning the specimen over at the end of the specified period of three minutes. To determine fine points in ratings below 50/0, the following symbols were designated:

25

#### Period with no wetting

or penetration

30

Symbol: 0+ ----- 2 to 30 seconds  
0+2 ----- 30 to 90 seconds  
0+3 ----- (1)

190 seconds to just below 3 minutes.

35

The 3M oil repellency test is based on the different penetrating properties of the two hydrocarbon liquids, Nujol (a water white heavy lubricating oil) and n-heptane. The Nujol-heptane proportions for each rating were selected by 3M so as to give oily stain resistance somewhat comparable to the water-borne stain resistance corresponding to each of the spray ratings of the AATCC Standard Test Method 22-1952:

45

|    | Oil Repellency Rating | Percent n-Heptane<br>(by volume) | Percent Nujol<br>(by volume) |
|----|-----------------------|----------------------------------|------------------------------|
| 50 | 100+                  | 60                               | 40                           |
|    | 100                   | 50                               | 50                           |
|    | 90                    | 40                               | 60                           |
|    | 80                    | 30                               | 70                           |
|    | 70                    | 20                               | 80                           |
|    | 50                    | 0                                | 100                          |

<sup>1</sup> No hold out to Nujol.

55

The standard oil-heptane mixture are contained in small stoppered medicine dropper bottles. A drop of each mixture is placed on the fabric to be tested. The appearance of the test oil is observed through the drop. Note whether wetting or penetration occurs. The number corresponding to that mixture containing the highest percentage of n-heptane which does not penetrate or wet the fabric after three minutes is considered the oil repellency rating of the system.

65

The change in the optical refractivity of the drop is often an indication of wetting. In some cases wetting can be determined better by observing the other side of the fabric. In some cases of "0" oil/heptane rating, the symbol "0+" has been used to indicate some resistance to wetting by oil.

#### Stain repellency (liquid stains)

The fabrics to be tested are stretched lightly on 12" x 31" frames. All or part of the frame area is used de-

pending upon the amount of the test fabric available. The frames are supported at both ends with the fabric about 8 inches above a black horizontal surface. The fabric touches nothing except the frame.

Three inch medicine droppers are used to draw the liquid stains from their containers. Each stopper is calibrated and marked on the exterior for a volume of one cubic centimeter. The liquid stain is squeezed vertically downward from a height of 2 inches above the cloth.

After five minutes the unabsorbed stain is wiped off the fabric with two sweeps of "Kleenex" tissue and the stains rated as follows:

| Appearance:                        | Stain rating |
|------------------------------------|--------------|
| Heavy stain over large area        | 1            |
| Heavy stain over medium sized area | 2            |
| Heavy stain over small area        | 3            |
| Medium stain over large area       | 4            |
| Medium stain over medium area      | 5            |
| Medium stain over small area       | 6            |
| Light stain over large area        | 7            |
| Light stain over small area        | 8            |
| Very slight visible stain          | 9            |
| No visible stain                   | 10           |

Duplicate sets of stains are applied in separate areas so that one-half of the fabric can be washed. Generally, the wash is carried out with 50 grams of "Fab," a cotton cycle, and a dummy load to total 5 pounds in a "Norge Home Automatic Washer."

#### WATER STAINS

1. Instant tea<sup>1</sup>
2. Blue-black ink
3. Grape juice
4. Salad mustard
5. Chocolate syrup

#### OIL STAINS

6. Salad oil
7. 20/20 motor oil
8. Oleomargarine<sup>2</sup>
9. Tomato sauce
10. Hand Lotion

<sup>1</sup> 8 cc. dry powder/200 cc. water applied @ 160° F.  
<sup>2</sup> Melted and applied at 160° F.

In all cases the stains are allowed to dry on the fabrics for twenty-four hours before washing.

#### Dry soil test

Fifteen to twenty 6" x 8" numbered specimens, usually 80 x 80 cotton, including at least one untreated control are tumbled for thirty minutes with 10 percent, based on the weight of the fabric of "Cyanamid Soil." The tumbling is carried out in a 5 liter capacity "Five Minute Home Cleaner" at 44 r.p.m. Six No. 8 neoprene rubber stoppers are distributed among the specimens to increase mechanical action. At the end of the tumbling, the specimens are removed and each shaken up and down fifteen times by hand to remove surface dirt.

The specimens are then cut to produce two pieces each 4" x 3". One half, i.e., one piece is washed with 50 grams of "Fab" in a cotton cycle with a five pound dummy load, then hung to dry and lightly ironed under a clean cotton cloth.

The degree of soil is determined with the "Photovolt Reflectance Meter" (Tri Blue filter). Six readings per specimen are made and the arithmetic average reported.

The "Cyanamid Soil" is prepared by blending the dry ingredients thoroughly. The blended dry ingredients are dried in a forced draft convection oven for eight hours at 50° C., then milled twenty-five hours with ceramic balls and stored in a polyethylene bag.

#### Dry soil ingredients

| Material:                           | Percent by weight |
|-------------------------------------|-------------------|
| Peat moss -----                     | 38                |
| Cement -----                        | 17                |
| Kaolin clay <sup>1</sup> -----      | 17                |
| Silica, 200 mesh <sup>2</sup> ----- | 17                |
| Furnace black <sup>3</sup> -----    | 1.75              |
| Red iron oxide <sup>4</sup> -----   | 0.50              |
| Mineral oil -----                   | 8.75              |
|                                     | 100.00            |

<sup>1</sup> R. T. Vanderbilt "Peerless" grade or equivalent.

<sup>2</sup> Davison Chemical Company.

<sup>3</sup> Benny and Smith Company, Molaceo.

<sup>4</sup> C. K. Williams Company.

In addition to the improved overall or total repellency exhibited by fabric treated with said polymers, the polymers are generally more heat, light and chemically stable than various fluoro chemical sizing agents known in the art.

Although the present invention has been described with reference to particular embodiments and examples, it will be apparent to those skilled in the art that variations and modifications of this invention can be made and that equivalents can be substituted therefor without departing from the principles and true spirit of the invention.

What is claimed is:

1. Fibrous organic material having affixed thereto in an amount sufficient to render said material resistant to water, oil, water-borne stains, oil-borne stains and dry soils, a polymer of a perfluoroalkylmethacrylate ester having the formula



where F is a fluorine and x is 1 to 20.

2. Cotton having affixed thereto a polymer in an amount sufficient to render the cotton repellent to particulate soil and reducing the residue of said particulate soil remaining after cotton and affixed polymer have been laundered in a conventional manner, and making said cotton and affixed polymer resistant to water, oil, water-borne stains, oil-borne stains and dry soils, said polymer-repellent comprising perfluoroalkylmethacrylate ester, said perfluoroalkylmethacrylate ester having the formula



where F is fluorine and x is 1 to 20.

3. Cotton in accordance with claim 2 wherein said polymer has an inherent viscosity in the range of about 0.2 to 3 and x is 2 to 12.

4. Cotton as defined in claim 2 wherein the perfluoro ester is pentadecafluoroctylmethacrylate.

5. A method of making fibrous organic material repellent to particulate soil and to reduce the residue of said particulate soil remaining on said fibrous material after laundering whilst making said fibrous material resistant to water, oil, water-borne stains, oil-borne stains and dry soils which comprises depositing a polymer of perfluoromethacrylate ester on said fibrous material, said ester having the formula:



where F is fluorine and X is 1 to 20, maintaining said treated fibrous material at a temperature in the range of room temperature to about 375° F. and obtaining treated fibrous material having a fluorine content in the range of 0.05 to 5 percent.

6. The method set forth in claim 5 wherein the treated fibrous material is air-dried and then cured at an elevated temperature up to about 375° F. for about five to sixty minutes.

7. A method as defined in claim 5 wherein the polymer is deposited by padding.

8. A method as defined in claim 5 wherein the polymer is deposited from a perfluoro organic solvent.

9. A method as defined in claim 5 wherein the polymer is deposited from an aqueous emulsion.

10. A method of making fibrous organic material substrate resistant to soiling by particulate soil and to reduce the residue of said particulate soil remaining on said fibrous material after laundering whilst making said fibrous material resistant to water, oil, water-borne stains, oil-borne stains and dry soils which comprises contacting said substrate, with an aqueous emulsion of polymeric perfluoroalkylmethacrylate ester, said ester having the formula:



where F is fluorine and X is 1 to 20 in amount to provide at least about 0.1 to about 10 percent by weight of said poly-perfluoroalkylmethacrylate based upon the weight of said substrate, separating the so-treated substrate from said aqueous emulsion and drying said treated substrate at a temperature in the range of room temperature to about 375° F.

11. A method of making fibrous organic material re-

sistant to soiling by particulate soil and to reduce the residue of said particulate soil remaining on said fibrous material after laundering whilst making said fibrous material resistant to water, oil, water-borne stains, oil-borne stains and dry soils which comprises contacting fibrous material hereinafter designated substrate, with a solution of a polymeric perfluoroalkylmethacrylate ester in perfluoro-organic solvent, said ester having the formula:

10



where F is fluorine and x is 1 to 20, separating the so-treated substrate from said perfluoro-organic solvent, and 15 curing said separated substrate at a curing temperature above room temperature and not in excess of about 375° F. to remove substantially all of said perfluoro-organic solvent.

12. The method set forth in claim 11 wherein the 20 perfluoro-organic solvent is bis-trifluoromethyl benzene.

#### References Cited

#### UNITED STATES PATENTS

25 2,642,416 6/1953 Ahlbrecht et al. \_\_\_\_ 260—83.5  
 3,102,103 8/1963 Ahlbrecht et al. \_\_\_\_ 260—29.6  
 3,282,905 11/1966 Fasick et al. \_\_\_\_ 260—89.5

WILLIAM D. MARTIN, Primary Examiner.

30 T. G. DAVIS, Assistant Examiner.